# EUROPEAN PATENT SPECIFICATION

(11) **EP 1 261 767 B1**
(45) Date of publication and mention of the grant of the patent: **28.09.2011**
(21) Application number: 01900895.2
(22) Date of filing: 05.01.2001
(51) Int. Cl.: D04H 13/00

(54) **COMPOSITE NONWOVEN FABRIC AND PROCESS FOR ITS MANUFACTURE**
VERBUNDWERKSTOFFE UND VERFAHREN ZUR HERSTELLUNG
TISSU COMPOSITE NON TISSE ET SON PROCEDE DE FABRICATION

(30) Priority: 06.01.2000 US 174750 P
(43) Date of publication of application: 04.12.2002
(73) Proprietor: Ahlstrom Nonwovens LLC, Windsor Locks, CT 06096 (US)
(72) Inventor: DUNCAN, Graham, Kirk, Duns, Berwickshire TD11 3DH (GB); MEIERHOEFER, Alan, William, Frederick MD 21701 (US); VOLPE, Raymond, Anthony, Wethersfield, CT 06109 (US)
(74) Representative: Mercer, Christopher Paul
(86) International application number: PCT/US2001/000320
(87) International publication number: WO 2001/049914

(56) References cited:
- EP-A- 0 492 554
- EP-A- 0 992 338
- US-A- 5 151 320

## Description

### Field of invention

This present invention relates to a process for the manufacture of composite fabrics. The invention relates especially to processes for the manufacture of composite fabrics in which a fibrous web that comprises wood-pulp fibers is joined to a spunlaid web, and to processes wherein the joining of the webs is effected by hydroentanglement.

### Background to the Intention

It has already been disclosed in US-A-5 151 320 (Homonoff et al) and US-A-5 573 841 (Adam et al) that a composite nonwoven material may be made by combining a spunbonded nonwoven and wood pulp by means of high-pressure water jets. However, it is inferred from the disclosure in these United States patents that a fully bonded spunbonded nonwoven is used and the strength properties of the resultant composite are similar to those of the spunbonded starting material.

### Summary of the Invention

The present invention provides a process for producing a composite nonwoven fabric comprising:
forming a first nonwoven web that comprises polymer filaments;
less than fully bonding the material of the first web, wherein the first web is less than fully bonded by thermal bonding, hydroentanglement, needle bonding, chemical bonding or adhesive bonding using bonding conditions that are less intensive than those used to achieve a fully bonded nonwoven material;
placing a second nonwoven web comprised of cellulose fibers adjacent to the first web, wherein the second nonwoven web is applied either as a pre-formed web or tissue or is formed on the first nonwoven web; and
joining the second web to the first web by fiber entanglement;
wherein the strength of the first web after bonding is no more than 35% of the strength of the composite fabric.

The filaments in the first web are preferably of man-made polymer.

For avoidance of doubt, it is declared that the expression "fiber entanglement" and the like herein include fiber-filament entanglement as well as fiber-fiber entanglement.

### Brief description of the drawing

Figure 1 is a graph illustrating addition of varying amounts of pulp to a minimally bonded base web and the total tensile strength of the resulting composite nowoven fabric.

### Description of exemplary embodiments

The said first web may be regarded as a base web. The base web material preferably comprises synthetic or other man-made filaments or fibers, in particular substantially continuous filaments. The base web material will generally comprise filaments or fibers made of a thermoplastic material, for example filaments or fibers of a polyamide, polyurethane, polyester or polyolefin, or a copolymer, e.g. block copolymer, containing olefin monomer units. The base web may also comprise, or consist of, bi-component or bi-constituent or mixed filaments or fibers. Suitable thermoplastic filamentary materials are disclosed in US-A-5 151 320 and US-A-5 573 841. In certain preferred embodiments, tho base web comprises polyester filaments, especially polyethylene terephthalate (PET) filaments, or polyolefin filaments, for example polyethylene or polypropylene filaments. Man-made cellulosic fibers, such as viscose rayon or lyocell fibers, may also come into consideration.

Of course, tho base web material may comprise a mixture of filaments or fibers of different materials, e.g., different thermoplastic materials. Furthermore, although in certain preferred embodiments the base web material will consist of, or consist essentially of, man-mado, especially synthetic, and more especially thermoplastic, filaments and/or fibers, the presence of other, non-interfering components is not precluded. The filaments or fibers will usually have a linear density of from 0.1 to 6 denier (0.0111 to 0.667 tox), e.g., from 0.3 to 4.6 denier (0.033 to 0.5 tex) and typically from 0.5 to 3.5 denier (0.056 to 0.389 tex).

The web is less than fully bonded sufficient for it to maintain its integrity during handling in the hydroentanglement process. Preferably, the bonding is effected by thermal bonding, although other bonding methods, such as hydroentanglement, needle bonding, chemical bonding or adhesive bonding, may come into consideration, instead of or in addition to the thermal bonding. In certain preferred embodiments, the base web is a spun-laid web.

Nonetheless, the base material in any embodiment is not be fully bonded. In general, such a material may be obtained by the normal methods for the production of bonded nonwoven materials with the modification that at least one of the usual bonding steps, e.g., the final bonding step, is omitted or carried out in a manner that is less intensive than normal, for example by using lower bonding temperatures, shorter bonding times, lower bonding pressures, lower entanglement energy inputs, lower needle density, lesser amounts of adhesive or other chemicals, or the like, as appropriate to the particular bonding method.

As one example spunlaid nonwovens or "spunbonded" materials are produced by bonding a spunlaid web by one or more techniques to provide fabric integrity. The spin laying of webs is disclosed, for example, in US-A-4 340 563 and US-A-3 692 618. In the production of spun-laid nonwovens or spunbonded materials, the bonding or consolidation operation is normally carried out by means of a thermal calendering process involving the application of heat and pressure to the unbonded web. Full or complete bonding of the web material is indicated by the characteristic that thermal calendering of the unbonded web material at increased temperatures and/or pressures does not improve the strength properties of the resulting web material. As an example a spunlaid web comprising polyethylene terephthalate filaments may be thermally calendered at a temperature below the melting point of the polymer (about 265°C) and at a "normal" pressure to produce a fully bonded nonwoven web. Naturally more than one combination of temperature and pressure will result in a fully bonded web material.

A less than-fully bonded spunlaid nonwoven material may be obtained by carrying out the thermal calendering process at a temperature that is lower than the melting point of the material from which the nonwoven has been made, for example lower than the softening point of that material and/or at a pressure below that normally used for that material. Thus, for example, the above spunlaid web comprising polyethylene terephthalate filaments may be thermally calendered at a temperature of from 80°C to 180°C, or more typically from 140°C to 160° C and at a pressure equal to, or more preferably less than, the above normal pressure to provide a less than fully bonded nonwoven wob material. It is believed that the thermals calendering temperature should exceed the glass transition temperature of the polymer used, for example 80°C in the case of polyethylene terephthalate. As would be expected the selection of a particular combination of material and thermal calendering temperature and pressure will result in a nonwoven web ranging from unbonded to fully bonded. The Invention is most advantageous with base web materials that have been less than fully bonded to a point sufficient only to provide for base web integrity until subsequent entanglement with the below-described second web.

The base web material, prior to the entanglement process, may optionally be subjected to cross stretching by at least 5 percent of its original extent, as described in US-A-5 151 320.

Prior to the entanglement process, the said second web, being a web comprising cellulose pulp fibers, is applied to the base web material. The web containing cellulose pulp fibers may be applied as a pre-formed web or tissue or may be formed on the base web material, for example by means of a wet-laying or air-laying process. The use of a pre-formed web (e.g. one formed by a wet-laying process) containing cellulose pulp fibers is currently preferred for manufacturing reasons. Ways in which a web comprising cellulose pulp fibers may be applied to a base web material are disclosed in the above-mentioned US-A-5 151 320 and US-A-5 673 841.

The cellulose pulp fibers may be derived from a wide range of naturally occurring sources of cellulose fibers, and are preferably wood pulp fibers (including hardwood pulp, soft wood pulp and mixtures thereof), although non-wood vegetable pulp fibers such as those derived from cotton, flax sisal, hemp, jute, esparto grass, bagasse, straw and abaca fibers may also come into consideration. Mixtures of various cellulose pulp fibers may also be used.

The cellulose pulp fibers, which may be used, include conventional short papermaking fibers, particularly having a fiber length of 25mm or less. The average fiber length is typically greater than 0.7mm and is most preferably from 1.5 to 5mm. Conventional papermaking fibers include the conventional papermaking wood pulp fibers produced by the well-known Kraft process.

Preferably said second web is formed entirely, or substantially entirely, of cellulose pulp fibers, and more preferably wood pulp. The second web may also comprise synthetic or other man-made fibers, for example in an amount of up to 50 percent by weight of the total fiber content of the cellulose fiber-containing web based on economic considerations. Synthetic or man-made fibers can be added in greater amounts to achieve other desired properties. Such man-made fibers include, for example, fibers made of rayon, polyester, polyolefin (e.g., polyethylene or polypropylene), polyamide (e.g., a nylon) or the like. Suitable man-made fibers include those having a fiber length of from about 3 to 25 mm and a denier per filament of 1.0 to 3.0 (0.111 to 0.333 tex).

The basis weights (grammages) of the first and second webs may be selected according to the fiber and/or filament constitution and the intended end use. The first web, e.g., a spunlaid nonwoven web, will have a basis weight of, in general, from 5 to 100, preferably from 15 to 90 and typicaly from 20 to 70, grams per square meter (gsm). The second web, for example, a web formed of wood pulp fibers, will have a basis weight of, in general, from 5 to 100, preferably from 10 to 80 and typically from 20 to 60, gsm

After assembly of the multi-layer structure comprising the base web material and the cellulose-fiber-containing web, the structure is subjected to a hydroentanglement operation, preferably a low to medium pressure hydroentanglement operation. Hydroentanglement operations are described in US-A-4 883 709 (Nozaki) and in US-A-5 009 747 (Viazmensky et al.). The hydroentanglament operation is preferably carried out by passing the multi-layer structure under a series of fluid streams or jots that directly impinge upon the top surface of the celluloso-fiber-containing layer with sufficient force to cause a proportion of the fibers therein, especially the short papermaking fibers, to be propelled into and entangled with the base web material. Preferably, a series or bank of jets is employed with the orifices and spacing between the orifices being substantially as disclosed in the aforesaid Nozakl patent or the Viazmensky et al. patent. The said fluid streams or jets are preferably streams or jets of an aqueous liquid.

As disclosed in the Viazmensky et al. patent, the total energy input provided by the fluid jets or streams may be calculated by the formula. $E = 0.125 YPG / bS$
Wherein Y = the number of orifices per linear inch of manifold width, P = the pressure in psig (pounds per square inch gauge) of liquid in the manifold, G = the volumetric flow in cubic feet per minute per orifice, S = the speed of the web material under the fluid jets or streams in feet per minute and b = the basis weight of the fabric produced in ounces per square yard. The total amount of energy, E, expended in treating the web is the sum of the Individual energy values for each pass under each manifold, if there is more than one manifold and/or if there is more than one pass. In general, the total energy input is from 0.07 to 0.4 horsepower-hours per pound (HPhr/Ib) (0.41 to 2.37 MJ/kg). Preferably, however, the total energy input is from 0.1 to 0.3 HPhr/Ib (0.59 to 1.78 MJ/kg), more preferably from 0.12 to 0.28 HPhr/Ib (0.71 to 1.66 MJ/kg).

The less than fully bonded nonwoven base web material having a low bond intensity that is employed, in accordance with the present invention would have been expected to provide a comparatively low-strength base for combining with the fibrous sheet or web that contains cellulose fibers. However, when the cellulose fibers are entangled into the incompletely bonded nonwoven material, it has surprisingly been found that the strength of the composite is significantly greater than that of the starting nonwoven base web material. Moreover, it has been found that the strength of the composite increases with higher pressures and/or higher energies used in the hydroentanglement process. Thus, if a less than-fully bonded spun-laid nonwoven material without the application of wood pulp and a comparable, less than-fully bonded spun-laid nonwoven material to which wood pulp has been applied are subjected to the same entanglement operation profile, the final strength of the nonwoven without the wood pulp is much lower than that of the nonwoven/wood pulp composite.

The beneficial effects of the wood pulp on the strength of the composite is unexpected because, first, there is no obvious mechanism whereby the cellulose may bond with the polymers used in the base web material (in particular PET or polypropylene) and, second, it is conceivable that the wood pulp would have acted to absorb energy from the entanglement, jets and hence reduce their effect on strength generation. With the use of more highly bonded base web materials, our studies have shown that, although the starting strength of the spunbonded material may be higher, it changes much less during the entanglement process.

Interestingly, for less than fully bonded base webs, not only is the strength of the composite after hydro-entanglement significantly increased over that of the same base web entangled on its own, but, if the wood pulp is subsequently removed from the final composite (for example by dissolving it with a suitable acid), the thus "regenerated" base web has a strength similar to that of the untreated, starting base web. Further, when a more fully bonded base web is used, similar removal of the wood pulp from the final composite again results in a "regenerated" base web that has strength properties very similar to those of the starting base web.

It has been found that for entangled composites of this invention the strength of the untreated base web contributes no more than 35%, of the final composite strength, in particular of the total tensile strength of the final composite. The strength may be measured, for example, as the tensile strength in the machine direction (MD) or cross direction (CD) or as the total tensile strength (sum of the MD+CD tensile strengths).

The composite nonwoven fabrics manufactured according to the present invention may find use in a variety of applications, for example, as molding substrates (e.g., in the automotive industry), as geotextiles, as wiping materials, both wet and dry, and in the medical field as disposable garments such as surgical gowns and drapes. Depending upon the intended end-use, the composite fabrics of the present invention may include, in addition to the above-discussed fibrous components, various other additives such as surfactants, fire retardants, pigments, liquid-repellants, super-absorbents, molecular sieves, and various other particulates such as starches, activated charcoal or clay.

The use of the present invention can give rise to products having excellent aesthetic qualities. Entanglement of pulp fibers and the like into conventional fully thermally bonded spunlaid nonwovens normally results in a non-uniform appearance. For example, the thermal bondpoints become exposed and give the impression of defects or pinholes or lack of integrity. However, by using a less-than-fully bonded spunlaid nonwoven in accordance with this invention it is possible to overcome that deficiency, and to do so with little or no detriment to the strength of the final composite nonwoven. Furthermore, it is also possible to produce composite nonwoven fabrics that have improved bulk, hand and absorbency. The inventive composite nonwoven fabrics can also be dried satisfactorily without the formation of cockles.

Having generally described the invention, the following examples are included for purposes of illustration so that the invention may be more readily understood and are in no way intended to limit the scope of the invention unless otherwise specifically specified.

### Example 1

A spunlaid base web having a nominal base weight of 30 gsm and comprising 100% PET 1-denier (0.111 tex) fibers was overlaid with a tissue in the form of a web comprising wood pulp fibers (Crofton ECH/Harmac K10S) containing approximately 38 gsm bone-dry fiber. The resultant multi-layer composite was then passed through a production-size hydroentanglement machine in which jets of water were directed at the tissue side of the said composite. Suction was applied from beneath the composite by means of vacuum boxes, in order to remove excess water.

Two different profiles of the water-jet apparatus were employed, which profiles are summarized in Table 1 hereinafter. In that Table, the column numbers 1 to 10 indicate the sequence of the nozzles. The figures in the "Bar" rows are the pressures employed, which are expressed in bar (1 bar = 10⁵ Pa or approximately 14.5 Ib-force/in²). The figures in the "Dia" rows are the nozzle diameters expressed in µm. The density of the 90 µm holes in the injectors was 2000 per meter (51 per inch) and the density of the 120 µm holes was 1666 per meter (45.2 per inch). The speed of the composite through the hydroentanglement machine was 46 meters per minute.

Furthermore, different grades of base web were used, the webs differing primarily in the temperature at which the thermal calendering operation was carried out. The base webs are identified as follows:

| | |
|---|---|
| Web 1: | Base web was bonded at 120°C. |
| Web 2: | Base web was bonded at 160°C. |
| Web 3: | Base web was bonded at 210°C and represents a reference, normally bonded material. |

The composite nonwoven fabrics obtained by hydroentanglement were tested for various physical properties and the results obtained are shown hereinafter. The test methods were:

| | | |
|---|---|---|
| Basis Weight | TAPPI | T410 |
| Tensile Strength | TAPPI | T494* |
| Elongation | TAPPI | T494* |
| Elemendorf Tear | TAPPI | T414 |

| | | |
|---|---|---|
| *using a strain rate of 300 mm/min. | | |

Table 2 shows the results for the said composite nonwoven fabrics under the heading "Base web + tissue", the particular web being identified at the top of each column of results. The entanglement profile used is shown below. Tests were also carried out on samples of the starting spunbonded base webs without the addition of the tissue, and the results obtained are also shown in Table 2, under the heading "Base web".

In addition, further trials were run in order to compare the results obtained for the starting base web, for the starting web after entanglement but without the tissue addition, and for the starting web subjected to entanglement with the tissue. The results from these trials are shown in Table 3 hereinafter. The results differ in certain respects from those recorded in Table 2. This is because the data was obtained from two different runs with slightly different machine settings; the natural variability of the materials also contributed to the differences.

| TABLE 1 | | | | | | | | | | | |
|---|---|---|---|---|---|---|---|---|---|---|---|
| Profile | Injector Number | | | | | | | | | | |
| | | 1 | 2 | 3 | 4 | 5 | 6 | 7 | 8 | 9 | 10 |
| 1 | Bar | 35 | 36 | 40 | 50 | 68 | 68 | 68 | 68 | 47 | 30 |
| | Dia | 90 | 90 | 90 | 90 | 90 | 90 | 90 | 90 | 90 | 90 |
| | | | | | | | | | | | |
| 2 | Bar | 6 | 30 | 50 | 60 | 70 | 80 | 85 | 85 | 85 | 80 |
| | Dia | 120 | 90 | 90 | 90 | 90 | 120 | 120 | 120 | 120 | 90 |

| TABLE 2 | | | | | | | |
|---|---|---|---|---|---|---|---|
| | Base Web + Tissue | | | | Base Web | | |
| | web 1 | web 2 | web 3 | web 2 | web 1 | web 2 | web 3 |
| Entanglement Profile | 1 | 1 | 1 | 2 | none | none | none |
| Basis Wt gsm | 76.1 | 75.3 | 73.1 | 73.9 | 30.7 | 32.3 | 25.2 |
| Dry Tensile, MD N/m | 2918 | 2628 | 2231 | 3059 | 111 | 511 | 890 |
| Dry Tensile, CD N/m | 1393 | 1085 | 956 | 1409 | 38 | 148 | 444 |
| Elmendorf Tear, MD mN | 11920 | 10520 | 5000 | 7080 | 10040 | 10240 | 4480 |
| Elmendorf Tear, CD mN | 13440 | 12480 | 6560 | 12160 | --- | --- | --- |
| Dry Elongation, MD (%) | 42 | 34.6 | 23.4 | 42.9 | 5.7 | 7.6 | 18.5 |
| Dry Elongation, CD (%) | 99.4 | 86.4 | 45.6 | 92.6 | 40.3 | 22.3 | 20.5 |

| TABLE 3 | | | | | | | | | |
|---|---|---|---|---|---|---|---|---|---|
| | Web 1 | | | Web 2 | | | Web 3 | | |
| Entanglement Profile | none | 1 | 1 | none | 1 | 1 | none | 1 | 1 |
| | web | web | web + tissue | web | web | web + tissue | web | web | web + tissue |
| Basis Weight gsm | 31 | 32 | 74 | 32 | 33 | 75 | 25 | 32 | 73 |
| Tensile MD N/m | 111 | 881 | 2548 | 511 | 204 | 2705 | 890 | 1138 | 2231 |
| Tensile CD N/m | 38 | 536 | 1429 | 148 | 272 | 1404 | 444 | 567 | 956 |
| Elmendorf MD MN | 10040 | 15720 | 13560 | 10240 | 14440 | 13520 | 4480 | 6040 | 5000 |

### Example 2

Three spunlaid base webs made from 100% polypropylene were used. Their basic characteristics were as follows:

| TABLE 4 | | | |
|---|---|---|---|
| | Web 4 | Web 5 | Web 6 |
| Nominal basis weight (gsm) | 28 | 28 | 28 |
| Fiber Diameter (Denier) | 1.0 | 1.5 | 2.2 |
| Bonding Temperature (°C) | 90 | 90 | 137 |

Web 6 represents a reference, normally bonded material.

These webs were each subjected to three different processing combinations as follows:
(a) A sample of each web was subjected to hydro-entanglement on Laboratory equipment using Profile 2 in Table 1 of Example 1. The samples were then dried.
(b) A sample of each web was overlaid with a tissue containing wood pulp fibers (Harmac K10) containing the equivalent of approximately 58 gsm of bone-dry fiber. The composites were then subjected to hydro-entanglement again using Profile 2 in Table 1 of Example 1 on a laboratory unit. The entangled composites were then dried.
(c) Duplicate samples, made according to (b) above, were placed in concentrated sulfuric acid (95%) at room temperature in order to etch out the wood pulp fibers. The concentration and nature of the acid was chosen so that it would have no effect on the polypropylene fibers. The thus "regenerated" web was then washed in water and dried.

The samples from all three processing conditions were then tested for tensile strength; the results are shown in Table 5.

| TABLE 5 | | | |
|---|---|---|---|
| | | Tensile MD N/m | Tensile CD N/m |
| Web 4 | untreated base web | 184 | 51 |
| | entangled base web | 118 | 88 |
| | entangled base web + tissue | 1644 | 508 |
| | regenerated baseweb | 71 | 0 |
| | Contribution To Composite From Untreated Baseweb | 11.2 % | 10.0 % |
| | | | |
| Web 5 | untreated base web | 103 | 59 |
| | entangled base web | 83 | 118 |
| | entangled base web + tissue | 1691 | 900 |
| | regenerated baseweb | 0 | 0 |
| | Contribution To Composite From Untreated Baseweb | 6.1 % | 6.6 % |
| | | | |
| Web 6 | untreated base web | 1103 | 758 |
| | entangled base web | 995 | 688 |
| | entangled base web + tissue | 1824 | 998 |
| | regenerated baseweb | 862 | 629 |
| | Contribution To Composite From Untreated Baseweb | 60.5 % | 76.0 % |

### Example 3

Three spunlaid basewebs made from 100% polypropylene were used. Their basic characteristics are listed in TABLE 6.

| TABLE 6 | | | |
|---|---|---|---|
| | Web 7 | Web 8 | Web 9 |
| Nominal basis weight (gsm) | 17 | 17 | 17 |
| Fiber Diameter (Denier) | 2.2 | 2.2 | 2.2 |
| Bonding Temperature (°C) | 128 | 110 | 137 |

Web 9 represents a reference, normally bonded material.

These webs were subjected to three different processing combination as follows:
(a) A sample of each web was subjected to hydro-entanglement on laboratory equipment using the profile given below in Table 7 and dried.

| TABLE 7 | | | | | | | | | | | |
|---|---|---|---|---|---|---|---|---|---|---|---|
| Profile | Injector Number | | | | | | | | | | |
| | | 1 | 2 | 3 | 4 | 5 | 6 | 7 | 8 | 9 | 10 |
| 3 | Bar | 15 | 30 | 40 | 50 | 60 | 60 | 60 | 60 | 60 | 60 |
| | Dia | 90 | 90 | 90 | 90 | 90 | 90 | 90 | 90 | 90 | 90 |

(b) A sample of each web was overlaid with a tissue containing wood pulp fibers (Harmac K10S) containing the equivalent of approximately 38 gsm of bone-dry fiber. The composites were than subjected to hydro-entanglement using the above Profile 3 on a laboratory unit. The entangled composites were then dried.
(c) Duplicate samples, made according to (b) above, were placed in concentrated sulfuric acid (95%) at room temperature in order to etch out the wood pulp fibers. The concentration and nature of the acid was chosen so that it would have no effect on the polypropylene fibers. The thus "regenerated" web was then washed in water and dried.

The samples from all three processing conditions were then tested for tensile strength, the results of which are shown in Table 8.

| TABLE 8 | | | |
|---|---|---|---|
| | | Tensile MD (N/m) | Tensile CD (N/m) |
| Web 7 | untreated base web | 273 | 227 |
| | entangled base web | 228 | 191 |
| | entangled base web + tissue | 941 | 504 |
| | regenerated baseweb | 324 | 106 |
| | Contribution To Composite From Untreated Baseweb | 29.0 % | 45.0 % |
| | | | |
| Web 8 | untreated base web | 306 | 174 |
| | entangled base web | 152 | 122 |
| | entangled base web + tissue | 1006 | 439 |
| | regenerated baseweb | 42 | 63 |
| | Contribution To Composite From Untreated Baseweb | 30.4 % | 39.6 % |
| | | | |
| Web 9 | untreated base web | 624 | 462 |
| | entangled base web | 556 | 383 |
| | entangled base web + tissue | 1026 | 643 |
| | regenerated baseweb | 780 | 478 |
| | Contribution To Composite From Untreated Baseweb | 60.8 % | 71.9% |

### Example 4

Two spunlaid base webs as in Example 1 and made from 100% polyester were used. Their basic characteristics are listed in TABLE 9.

| TABLE 9 | | |
|---|---|---|
| | Web 2 | Web 3 |
| Nominal basis weight (gsm) | 30 | 30 |
| Fiber diameter (denier) | 1.0 | 1.0 |
| Bonding temperature (°C) | 160 °C | 210 °C |

Web 3 represents a reference, normally bonded material.

These webs were subjected to three different processing combinations as follows:
(a) A sample of each web was subjected to hydro-entanglement on a laboratory unit using Profile 1 in Table 1 of Example 1. The samples were then dried.
(b) Each web was overlaid with a tissue containing wood pulp fibers (Harmac K10S) containing the equivalent of approximately 38 gsm of bone-dry fiber. The composites were then subjected to hydro-entanglement using the said Profile 1 on a laboratory unit. The entangled composites were then dried on steam-filled cans.
(c) Duplicate samples, made according to (b) above, were placed in concentrated sulfuric acid (75%) at room temperature in order to etch out the wood pulp fibers. The concentration and nature of the acid was chosen so that it would have no effect on the polyester fibers. The thus "regenerated" web was then washed in water and dried.

The samples from all three processing conditions were then tested for tensile strength, the results of which are show in Table 10.

| TABLE 10 | | | |
|---|---|---|---|
| | | Tensile MD (N/m) | Tensile CD (N/m) |
| Web 2 | untreated base web | 468 | 149 |
| | entangled base web | 204 | 272 |
| | entangled base web + tissue | 1944 | 773 |
| | regenerated baseweb | 247 | 75 |
| | Contribution To Composite From Untreated Baseweb | 24.1 % | 19.3 % |
| | | | |
| Web 3 | untreated base web | 890 | 444 |
| | entangled base web | 1138 | 567 |
| | entangled base web + tissue | 1853 | 921 |
| | regenerated baseweb | 956 | 448 |
| | Contribution To Composite From Untreated Baseweb | 48.0 % | 48.2 % |

### Example 5

Previously described Web 2 was used for this example. Samples were prepared as follows:
(a) Layers of wood pulp of varying weights were combined with samples of web 2 by forming the wood pulp layers directly onto the baseweb using standard wetlaying handsheet mold apparatus. Woodpulp additions were from nominally 5 gsm to nominally 40 gsm of bone-dry fiber. The fiber used was Harmac K10S; it was dispersed in a standard laboratory pulper but was given no additional processing (such as refining or beating).
(b) Duplicate samples of each weight addition of (a) above were subjected to hydro-entanglement using Profile 1 in Table 1 of Example 1 on a laboratory unit. The entangled composites were then dried.
(c) Separate sheets of wood pulp only at the same nominal weights as (a) above were made and dried.

Four separate samples each of the woodpulp sheets, wood pulp/baseweb sheets and hydroentangled wood pulp/baseweb composite tested for basis weight and tensile strength. The average results for each are shown in Table 11 and graphically in Figure 1.

As a result of hydro-entangling as little as 5 gsm of wood pulp into the baseweb, the strength of the baseweb is increased by a surprisingly large amount, i.e., the total tensile strength increases from 659 N/m in the baseweb alone to 1461 N/m after entanglement with 5 gsm of woodpulp (baseweb contributing only 45% of the final strength).

| TABLE 11 | | | | | | | | | | |
|---|---|---|---|---|---|---|---|---|---|---|
| sample | property | nominal weight of woodpub addition (gsm) | | | | | | | | |
| | | 0 | 5 | 10 | 15 | 20 | 25 | 30 | 35 | 40 |
| | | | | | | | | | | |
| woodpulp | basis weight (gsm) | N/A | 5.5 | 8.7 | 15.5 | 49.6 | 24.0 | 29.3 | 34.0 | 38.6 |
| | total tensile strength (N/m) | N/A | 71 | 138 | 467 | 576 | 739 | 955 | 999 | 1179 |
| | | | | | | | | | | |
| Web 2 + woodpulp | basis weight (gsm) | 32.3 | 37.7 | 40.3 | 44.2 | 50.0 | 54.2 | 59.5 | 66.3 | 71.2 |
| | total tensile strength (N/m) | 659 | 744 | 785 | 899 | 1177 | 1061 | 1345 | 1861 | 2086 |
| | | | | | | | | | | |
| entangled Web 2 + woodpulp | basis weight (gsm) | N/A | 36.6 | 40.4 | 45.8 | 50.5 | 54.7 | 58.9 | 65.0 | 71.4 |
| | total tensile strength (N/m) | N/A | 1461 | 2069 | 2206 | 2566 | 2583 | 2647 | 2817 | 3263 |

## Claims

1. A process for producing a composite nonwoven fabric comprising:
forming a first nonwoven web that comprises polymer filaments;
less than fully bonding the material of the first web, wherein the first web is less than fully bonded by thermal bonding, hydroentanglement, needle bonding, chemical bonding or adhesive bonding using bonding conditions that are less intensive than those used to achieve a fully bonded nonwoven material;
placing a second nonwoven web comprised of cellulose fibers adjacent to the first web, wherein the second nonwoven web is applied either as a pre-formed web or tissue or is formed on the first nonwoven web; and
joining the second web to the first web by fiber entanglement;
wherein the strength of the first web after bonding is no more than 35% of the strength of the composite fabric.

2. The process of claim 1 wherein the first nonwoven web is less than fully bonded by thermal bonding.

3. The process of claim 1 wherein the first nonwoven web is less than fully bonded by thermal calendering at a temperature bellow a melting point or a softening point of the filaments.

4. The process of any preceding claim comprising the step of wet laying cellulose fibers to form the second web.

5. The process of any one of claims 1 to 3 comprising the step of wet laying or air laying cellulose fibers on the first web two form the second web.

6. The process of any preceding claim comprising the step of wet laying the cellulose fibers to form the second web prior to the step of placing the second web adjacent to the first web.

7. The process of any preceding claim wherein the step of joining comprises hydroentanglement of the fibers of the second web into the first web at a total entanglement energy input in the range of 0.07 to 0.4 horsepower-hours per pound (0.41 to 2.37 MJ/kg).

8. The process of any preceding claim wherein the first web comprises spunlaid filaments.

9. The process of any preceding claim wherein the first web comprises spunlaid filaments of a material selected from the group consisting of polyethylene terephthalate, polypropylene and mixtures thereof.

10. The process of any preceding claim wherein the first web consists of thermoplastic filaments having a denier in the range of 0.5 to 2.5 (linear density of 0.56 to 2.78 dtex).

11. The process of any preceding claim wherein the first web material comprises at least one of bicomponent filaments, bicomponent fibres, biconstituent filaments and biconstituent fibres.

12. The process of any preceding claim wherein the second web contains man-made fibers in an amount up to 50% by weight of the total fiber content of the second web.

## Patentansprüche

1. Verfahren zur Herstellung eines Nonwoven-Verbundgewebes, umfassend:
Bilden einer ersten Nonwoven-Bahn, die Polymerfilamente umfasst;
nicht ganz vollständiges Verbinden des Materials der ersten Bahn, wobei die erste Bahn durch thermisches Verbinden, Hydroverknäuelung, Nadelverbinden, chemisches Verbinden oder Klebverbinden unter Anwendung von Verbindungsbedingungen, die weniger intensiv sind als diejenigen, die zur Erzielung eines vollständig verbundenen Nonwoven-Materials angewandt werden, nicht ganz vollständig verbunden wird;
Platzieren einer zweiten Nonwoven-Bahn_{;} die aus Zellulosefasern aufgebaut ist, angrenzend an die erste Bahn, wobei die zweite Nonwoven-Bahn entweder als zuvor gebildete Bahn oder Textilgewebe aufgebracht wird oder auf der ersten Nonwoven-Bahn gebildet wird; und
Verknüpfen der zweiten Bahn mit der ersten Bahn durch Faserverknäuelung;
wobei die Festigkeit der ersten Bahn nach dem Verbinden nicht mehr als 35 % der Festigkeit des Verbundgewebes beträgt.

2. Verfahren gemäß Anspruch 1, wobei die erste Nonwoven-Bahn durch thermisches Verbinden nicht ganz vollständig verbunden wird.

3. Verfahren gemäß Anspruch 1, wobei die erste Nonwoven-Bahn durch thermisches Kalandrieren bei einer Temperatur unterhalb eines Schmelzpunktes oder eines Erweichungspunktes der Filamente nicht ganz vollständig verbunden wird.

4. Verfahren gemäß einem beliebigen der vorausgehenden Ansprüche, umfassend den Schritt des Nassverlegens von Zellulosefasern zur Bildung einer zweiten Bahn.

5. Verfahren gemäß einem der Ansprüche 1 bis 3, umfassend den Schritt des Nassverlegens oder Luftverlegens bzw. Airlayings von Zellulosefasern auf der ersten Bahn zur Bildung der zweiten Bahn.

6. Verfahren gemäß einem beliebigen der vorausgehenden Ansprüche, umfassend den Schritt des Nassverlegens der Zellulosefasern zur Bildung der zweiten Bahn vor dem Schritt des Platzierens der zweiten Bahn angrenzend an die erste Bahn.

7. Verfahren gemäß einem beliebigen der vorausgehenden Ansprüche, wobei der Schritt des Verknüpfens die Hydroverknäuelung der Fasern der zweiten Bahn in die erste Bahn bei einer Gesamtverknäuelungs-Energiezufuhr im Bereich von 0,07 bis 0,4 Pferdestärken pro Pfund (0,41 bis 2,37 MJ/kg) umfasst.

8. Verbundgewebe gemäß einem beliebigen der vorausgehenden Ansprüche, wobei die erste Bahn Spinnvlies-Filamente umfasst.

9. Verbundgewebe gemäß einem beliebigen der vorausgehenden Ansprüche, wobei die erste Bahn Spinnvlies-Filamente eines Materials umfasst, das aus der Gruppe gewählt ist, die aus Polyethylenterephthalat, Polypropylen und Mischungen davon besteht.

10. Verbundgewebe gemäß einem beliebigen der vorausgehenden Ansprüche, wobei die erste Bahn aus thermoplastischen Filamenten mit einem Denier im Bereich von 0,5 bis 2,5 besteht (lineare Dichte von 0,56 bis 2,78 dtex).

11. Verbundgewebe gemäß einem beliebigen der vorausgehenden Ansprüche, wobei das erste Bahnmaterial mindestens eines von Zweikomponentenfilamenten, Zweikomponentenfasern, aus zwei Bestandteilen bestehenden Filamenten und aus zwei Bestandteilen bestehenden Fasern umfasst.

12. Verbundgewebe gemäß einem beliebigen der vorausgehenden Ansprüche, wobei die zweite Bahn künstliche Fasern in einer Menge von bis zu 50 Gew.-% des Gesamtfasergehalts der zweiten Bahn enthält.

## Revendications

1. Procédé pour la production d'un nontissé composite comprenant :
la formation d'un premier voile non tissé qui comprend des filaments de polymère ;
le liage non total de la matière du premier voile, dans lequel le premier voile est non totalement lié par thermoliage, hydro-enchevêtrement, aiguilletage, liage chimique ou liage par adhésif à l'aide de conditions de liage qui sont moins sévères que celles utilisées pour réaliser une matière non tissée totalement liée ;
l'apposition d'un second voile non tissé constitué de fibres de cellulose adjacent au premier voile, dans laquelle le second voile non tissé soit est appliqué sous forme d'un voile ou tissu préformé soit est formé sur le premier voile non tissé ; et
le rattachement du second voile au premier voile par enchevêtrement de fibres ;
dans lequel la résistance du premier voile après liage n'est pas supérieure à 35 % de la résistance du tissu composite.

2. Procédé selon la revendication 1 dans lequel le premier voile non tissé est non totalement lié par thermoliage.

3. Procédé selon la revendication 1 dans lequel le premier voile non tissé est non totalement lié par calandrage thermique à une température au-dessous d'un point de fusion ou d'un point de ramollissement des filaments.

4. Procédé selon l'une quelconque des revendications précédentes comprenant l'étape de dépôt de fibres de cellulose en voie humide pour former le second voile.

5. Procédé selon l'une quelconque des revendications 1 à 3 comprenant l'étape de dépôt en voie humide ou de dépôt aérodynamique de fibres de cellulose pour former le second voile.

6. Procédé selon l'une quelconque des revendications précédentes comprenant l'étape de dépôt des fibres de cellulose en voie humide pour former le second voile avant l'étape d'apposition du second voile adjacent au premier voile.

7. Procédé selon l'une quelconque des revendications précédentes dans lequel l'étape de rattachement comprend l'hydro-enchevêtrement des fibres du second voile dans le premier voile avec un apport total d'énergie d'enchevêtrement dans la plage de 0,07 à 0,4 cheval-vapeur-heure par livre (0,41 à 2,37 MJ/kg).

8. Tissu composite selon l'une quelconque des revendications précédentes dans lequel le premier voile comprend des filaments formés en voie fondue (spunlaid).

9. Tissu composite selon l'une quelconque des revendications précédentes dans lequel le premier voile comprend des filaments formés en voie fondue d'une matière choisie dans le groupe constitué par le poly(téréphtalate d'éthylène), le polypropylène et les mélanges de ceux-ci.

10. Tissu composite selon l'une quelconque des revendications précédentes dans lequel le premier voile est constitué de filaments thermoplastiques ayant un denier dans la plage de 0,5 à 2,5 (une masse linéique de 0,56 à 2,78 dtex).

11. Tissu composite selon l'une quelconque des revendications précédentes dans lequel la matière du premier voile comprend au moins un constituant parmi les filaments bicomposés, les fibres bicomposées, les filaments biconstitués et les fibres biconstituées.

12. Tissu composite selon l'une quelconque des revendications précédentes dans lequel le second voile contient des fibres synthétiques en une quantité allant jusqu'à 50 % en poids de la teneur totale des fibres du second voile.
